

Feb. 13, 1945.

H. L. MEAD ET AL

2,369,311

FLOTATION OF ACIDIC MINERALS

Filed Oct. 12, 1942

FIG. 1.  
(PRIOR ART)



FIG. 2.



INVENTORS  
HARRY L. MEAD,  
ERNEST J. MAUST,

BY  
Elmer W. Harmon  
ATTORNEY

## UNITED STATES PATENT OFFICE

2,369,311

## FLOTATION OF ACIDIC MINERALS

Harry L. Mead and Ernest J. Maust, Brewster,  
Fla., assignors to American Cyanamid Company,  
New York, N. Y., a corporation of Maine

Application October 12, 1942, Serial No. 461,766

3 Claims. (Cl. 209—166)

This invention relates to the concentration of minerals by froth flotation, more particularly to the beneficiation of ores by floating acidic gangue therefrom.

Beneficiation of ores by froth flotation, using a cationic-type reagent to float one or more components from the residue has become a well known procedure. In some cases, an operation of this type has a definite advantage over the use of an anionic-type reagent to float the mineral values away from the gangue. This is particularly true in those cases where the anionic reagents suitable for use with the mineral to be concentrated are not sufficiently selective. In such cases, although good recoveries can be made, it is difficult to produce a concentrate of high grade. This difficulty very commonly appears, for example, in the beneficiation of non-sulfide ores containing silica-bearing gangue such as silica, or silicates such as mica and the like minerals.

Phosphate ores, such as Florida pebble phosphate, are typical of the non-sulfide ores which are readily adapted to beneficiation with these reagents. Accordingly, that ore will be used as illustrative in setting forth the process of the present invention. The invention, however, is not so limited. It may be equally well applied to the beneficiation of any ore in which an acidic gangue is to be floated from the mineral values. Among the ores which can be treated according to the process of the present invention are those in which the acidic mineral is to be separated from ores such as limestone, bauxite, barytes, ilmenite, calcite and the like. The process is equally applicable whether the acidic mineral is being concentrated as gangue or as product.

The invention will be more fully illustrated in connection with the following drawing which is thought to be substantially self-explanatory and in which:

Figure 1 represents a flow sheet of a typical process of the prior art; and,

Figure 2 represents a flow sheet showing the modified procedure of the present invention.

The use of cationic-type reagents in concentrating acidic gangue is not new per se, being well illustrated for example in U. S. Patent No. 2,205,503. The actual practice of such a process is relatively simple. In its general form, such practice is diagrammatically set forth in the flow scheme of Figure 1. As shown in Figure 1, the ore to be beneficiated is ground, deslimed to the necessary degree, pulped with water, the pulp conditioned with the reagent and then subjected to

10 froth flotation, whereby the acidic gangue is concentrated and collected. The froth concentrate is usually passed to a second machine and given a cleaner flotation without the use of additional reagents, although such reagents may be added if necessary. The middlings from this cleaner float are ordinarily small in quantity and can be either discarded or optionally recycled to the rougher flotation according to their mineral content.

As a process, this beneficiation procedure appears to be both simple and effective. Actually, it suffers from a number of practical drawbacks. First, the reagent cost, on the basis of the weight 15 of ore being treated, as compared with that for anionic-type reagents is high. The principal advantage of cationic reagents lies in their ability to produce a higher grade product having an increased net value despite the increased reagent cost. This advantage can be obtained only when the cationic flotation is carefully controlled to take the fullest possible advantage of the concentrating power of the cationic reagent.

Secondly, cationic-type reagents are not perfectly selective. In other words, cationic reagents, like the anionic-type, can not be depended upon to make an exact separation of the desirable and the undesirable materials. This fact presents a particularly serious drawback in the 20 case of cationic-type reagents. Not only is there a direct loss of potential product, but so much of the reagent as is used in floating this potential product is also wasted so far as performing useful work is concerned. These combined effects 25 may so increase the net cost of producing a higher grade product, that any economic advantage therefrom is lost. The losses may in some cases be great enough to place the cationic reagent at a disadvantage.

30 In the use of these cationic reagents, the presence of slimes is also very troublesome. For example, in the beneficiation of phosphate ores the presence of even a small fraction of one percent of slimes in the feed may increase the reagent 35 consumption to a point at which the operation is economically undesirable. In many cases, the presence of excessive slimes may render the process inoperative. As a consequence, the feed must be very thoroughly deslimed. This adds to the 40 cost of the operation and increases the necessity for obtaining the maximum benefit of the reagent's concentrating power.

45 In those operations, such as the beneficiation of phosphate ore, in which the unit profit is small these considerations are specially impor-

tant. The premium for high grade is relatively important as compared with the base price. A change in the net value of the product of even a few cents per ton may make the difference between a process which is commercially desirable and one which is not. Any loss in potential concentrating power of the reagents is aggravated by the tremendous production rate of an even relatively small operation.

In the ordinary practice, an attempt is therefore made to balance the amount of reagent used, and consequently the amount of gangue removed from a given amount of feed, against the loss of salable product with the gangue. It is economically advantageous to increase the removal of silica up to a certain optimum. Any additional improvement in grade is made at the expense of increased losses in product which in turn offset the economic advantages of producing a higher grade.

As a result, the cationic reagent is usually used in such a way that neither the maximum improvement in grade nor the maximum potential recovery is obtained. In the case of phosphate ores, for example, the demand for high grade product places the emphasis on grade rather than recovery. As a result considerable phosphate is lost by being carried off in the silica rougher concentrate. Part of this potentially salable product is recovered by retreating the middlings. Nevertheless, an appreciable quantity of salable product which it is highly desirable to recover is lost in the silica cleaner concentrate.

It is, therefore, an object of the present invention to establish a procedure by which a maximum utilization of the concentrating power of the reagent and a maximum recovery of salable product are more nearly realized. The present invention is particularly concerned with obtaining the maximum recovery of useful product, without a sacrifice in grade.

Surprisingly enough, the object of the present invention is accomplished by going contra to established practice. The present practice, as shown in Figure 1, is to add all the feed during the rougher flotation and subsequently clean the silica concentrate. According to the present invention, as shown in Figure 2, instead of feeding all the material to the rougher flotation machine, an appreciable quantity is added to the cleaner circuit. This greatly increases the physical quantity of middlings which are then utilized as a part of the feed to the rougher flotation.

Also, as shown in Figure 2, instead of basing the amount of reagent on the usual economic balance, the process contravenes the usual practice by using an excess of reagent to carry out the rougher concentration. As a result of combining what the art has taught to be a waste of reagent with what has been considered a reversal of the necessary feeding procedure, the amount of potentially useful product in the cleaner concentrate may be greatly reduced. Losses of product are reduced by as much as 35-50% below those obtainable by the best conventional practice.

Although the present invention is not intended to be limited by any particular theory of operation it is believed that the improved result is due to a combination of several factors. First, a considerable amount of excess reagent, over that which is used in the conventional practice, is employed in the rougher flotation. This enables the production of an excellent gangue con-

centration. However, as a result, the froth concentrate also contains a considerable quantity of unused reagent. Instead of losing any reagent removed in the froth, as in the prior practice, it is quickly utilized in floating a part of the easily floatable gangue from the fresh feed added during the cleaner flotation.

In addition, an appreciable amount of reagent is used up by reacting with the basic mineral, whereby the charge on a part of the product mineral is neutralized or reversed and these product particles are floated out in the froth concentrate. However, the reagent normally has a greater affinity for an acidic gangue than for the product. Accordingly, when this abnormally charged portion of the product is brought into contact with the large amount of easily floatable gangue in the fresh feed during the cleaner flotation, it undergoes another charge transfer. The reagent leaves the abnormally charged particles and is utilized in floating additional gangue. The now normally charged product particles settle out in the middlings and are recovered. Product losses in the cleaner concentrate are thereby reduced.

In addition to these direct recoveries, another factor adds to the overall efficiency of the entire process. As was noted above, because a part of the feed is added to during the cleaner flotation, the amount of middlings is increased. Adding these middlings to the rougher flotation results in an amount of material equal to this increase being subjected to flotation for longer than the normal length of time. Because of this increased time, the rougher flotation can produce an even better separation.

In addition, a further advantage is obtained because a part of the gangue content has already been removed before the total feed reaches the rougher flotation stage. Consequently, a greater quantity of feed may be treated for an equal amount of gangue to be removed. This enables a greater total through-put for a fixed amount of equipment and results in a greater overall efficiency.

Expressed in other terms, this advantage of the process of the present invention means that a greater amount of gangue may be concentrated with a fixed amount of reagent. For example, in beneficiating phosphate ore, using a fixed amount of reagent, as much as twenty percent or more of gangue can be concentrated.

The term "cationic reagents" as used in the present specification and claims is intended to include the general class of such compounds having large, positively charged surface-active ions, many of which have become known as promoters for the flotation of acidic gangue. These positively-charged ions are usually of relatively large size and weight and usually contain at least one amine, ammonium or other "onium" group.

Examples, for illustrative purposes only, of the commonly used reagents of this type include amines such as the lauryl or octadecyl amines and the like. Similarly, use has been made of the readily ionized amine salts such as the hydrochloride, acetate and the like. Other examples include, for example, quaternary compounds such as cetyl pyridinium bromide or chloride, lauryl trimethyl ammonium chloride or iodide and the like. Still another well known type includes compounds, such compounds as the polyalkylene polyamines, their condensation products with fatty acids and the salts thereof.

75 The process of the present invention can not

be readily limited as to the proportion of the total feed which should be added to the circuit in the cleaner stage. The amount required will obviously vary with circumstances, being dependent not only upon the nature and conditions of the ore but also upon the particular reagent being used. The critical factor appears to be the proportion of the gangue in the feed which, principally due to its size, is easily floatable. For the optimum results it is necessary to add enough fresh feed to the cleaner stage so that a sufficient amount of this easily floatable portion of the gangue will be available to use up the excess reagent and effect the charge transference. This will again obviously vary with circumstances, being particularly affected by changes in the nature of the ore, the efficiency of the grinding, the extent of desliming and other pre-treating processes.

Fortunately, however, the process is not critical as to the upper limit of the amount of material which may be added. A considerable excess of material over and above that necessary for the optimum result, may be present without adversely affecting the entire process. This can be taken advantage of by adding more than enough feed in the cleaner stage so that there will be present at all times enough easily floatable gangue to take care of the exceptional circumstances. In fact, as pointed out above, there is a certain advantage in adding as much feed at this point as can be done without effecting the final grade. Addition of fresh feed in this way increases the total overall recovery at a rate faster than the corresponding decrease in grade over a considerable range.

While the above discussion has been largely limited to phosphate beneficiation from ores containing a siliceous gangue, this was only because such ores are typical of the types which can be advantageously treated according to the process of the present invention. Because they are typical, phosphate ores will be used to illustrate the invention in the following examples in which all parts are by weight unless otherwise noted.

#### EXAMPLE 1

As illustrated of the prior art procedures 500 parts of a Florida pebble phosphate ore, assaying 31.63% B. P. L., which had been previously deslimed, polished and very thoroughly deslimed were pulped with 2300 parts of water. 0.72 lb./t. of a mixed polyethylene polyamine flotation reagent were added as a 2% solution, the mixture was passed to a Fagergren flotation machine, conditioned for 3 seconds and the silica concentrate removed. The silica concentrate was passed to a second Fagergren flotation machine, agitated for one second and the silicate cleaner concentrate removed. The results are shown in Table I.

Table I

| Phosphate tailing |                |     | Middling         |     | Silica concentrate |     | Phosphate overall recovery, percent |
|-------------------|----------------|-----|------------------|-----|--------------------|-----|-------------------------------------|
| Percent B. P. L.  | Percent insol. | Wt. | Percent B. P. L. | Wt. | Percent B. P. L.   | Wt. |                                     |
| 78.20             | .80            | 169 | 62.60            | 18  | 4.48               | 313 | 91.0                                |

#### EXAMPLE 2

The procedure of Example 1 was repeated but 174 parts of fresh feed were added in the cleaner

circuit. 140 parts of middlings were obtained. The results are shown in Table II.

Table II

| Percent B. P. L. | Percent insol. | Wt. | Phosphate tailing |      | Middling         |       | Silica concentrate |      | Phosphate overall recovery, percent |
|------------------|----------------|-----|-------------------|------|------------------|-------|--------------------|------|-------------------------------------|
|                  |                |     | Percent B. P. L.  | Wt.  | Percent B. P. L. | Wt.   | Percent B. P. L.   | Wt.  |                                     |
|                  |                |     | 78.18             | 1.10 | 162              | 51.65 | 140                | 2.82 | 372                                 |

It will be noted that in this test a total of 372 parts of silica concentrate was floated, this being 39 parts or 18.8% more than was floated in Example 1, using the same amount of reagent in both cases.

#### EXAMPLE 3

The procedure of Example 2 was repeated, adding 264 parts of feed to the cleaner flotation. The results are shown in Table III.

Table III

| Percent B. P. L. | Percent insol. | Wt. | Phosphate tailing |      | Middling         |       | Silica concentrate |      | Phosphate overall recovery, percent |
|------------------|----------------|-----|-------------------|------|------------------|-------|--------------------|------|-------------------------------------|
|                  |                |     | Percent B. P. L.  | Wt.  | Percent B. P. L. | Wt.   | Percent B. P. L.   | Wt.  |                                     |
|                  |                |     | 77.81             | 1.60 | 166              | 49.95 | 224                | 2.49 | 374                                 |

With the additional amount of feed added to the cleaner cell in this test, a total of 374 parts of silica concentrate was floated, representing 61 parts or 19.4% more than floated in Example 1 using identical amounts of reagent.

#### EXAMPLE 4

The procedure of Example 1 was repeated substituting 0.28 lb./t. of Armour amine hydrochloride (approximately C<sub>18</sub>) fed as an emulsion comprising 1.5 parts of the amine hydrochloride, 2 parts of a higher aliphatic alcohol frother (approximately C<sub>1</sub>-C<sub>8</sub>) and 72 parts of water. No feed was added in the cleaning circuit. The results are shown in Table IV.

Table IV

| Percent B. P. L. | Percent insol. | Wt. | Phosphate tailing |      | Middling         |       | Silica concentrate |      | Phosphate overall recovery, percent |
|------------------|----------------|-----|-------------------|------|------------------|-------|--------------------|------|-------------------------------------|
|                  |                |     | Percent B. P. L.  | Wt.  | Percent B. P. L. | Wt.   | Percent B. P. L.   | Wt.  |                                     |
|                  |                |     | 77.89             | 2.30 | 170              | 59.50 | 14                 | 4.48 | 302                                 |

#### EXAMPLE 5

Example 4 was repeated adding 180 parts of feed in the cleaner stage. The results are shown in Table V.

Table V

| Percent B. P. L. | Percent insol. | Wt. | Phosphate tailing |      | Middling         |       | Silica concentrate |      | Phosphate overall recovery, percent |
|------------------|----------------|-----|-------------------|------|------------------|-------|--------------------|------|-------------------------------------|
|                  |                |     | Percent B. P. L.  | Wt.  | Percent B. P. L. | Wt.   | Percent B. P. L.   | Wt.  |                                     |
|                  |                |     | 76.91             | 2.70 | 169              | 50.41 | 140                | 3.61 | 371                                 |

It is also to be noted in this test that 371 parts of silica concentrate was obtained, this being 69 parts or 22.8% more than was obtained in Example 4, using the same amount of reagent in both cases.

We claim:

1. In those processes of beneficiating ores by froth flotation in which an acidic mineral is floated from a non-acidic mineral by the aid of a cationic-type promoter the improvements which comprise the steps of dividing the feed into a major and a minor fraction; subjecting the major portion of the feed to a rougher flotation in the presence of a sufficient excess of promoter to insure an underflow sufficiently low in acidic mineral content, whereby the excess promoter and a normally excessive amount of non-acidic mineral are carried off in the overflow; subjecting the rougher flotation overflow to a cleaner flotation together with the minor fraction of the feed, said minor fraction of the feed being sufficient to insure the utilization of the excess promoter and the settling of substantially all of the non-acidic mineral content of the rougher flotation overflow, and returning the underflow from the cleaner flotation to the rougher flotation circuit.
2. In those processes of beneficiating ores by froth flotation in which the gangue is floated away from the mineral by the aid of a cationic-type promoter the improvements which comprise dividing the feed into a major and a minor fraction, subjecting the major fraction to a rougher flotation in the presence of a sufficient amount of a cationic-type promoter to insure an underflow sufficiently low in gangue, whereby a normally excessive amount of mineral and the excess pro-

5 moter is carried off in the rougher flotation over-  
flow, subjecting the rougher flotation overflow together with the minor fraction of the feed to a cleaner flotation, said minor fraction of feed being sufficient to insure the utilization of the ex-  
cess promoter and the settling of substantially all the mineral in the rougher flotation overflow, and returning the cleaner flotation underflow to the rougher flotation feed.

- 10 3. In those processes of beneficiating phos-  
phate ores by froth flotation in which the silica-  
bearing gangue is floated away from the mineral by the aid of a cationic-type promoter the im-  
provements which comprise dividing the feed into a major and a minor fraction, subjecting the ma-  
jor fraction to a rougher flotation in the presence  
15 of a sufficient amount of a cationic-type promoter  
to insure an underflow sufficiently low in silica-  
bearing gangue, whereby a normally excessive  
amount of mineral and the excess promoter is  
20 carried off in the rougher flotation overflow, sub-  
jecting the rougher flotation overflow together  
with the minor fraction of the feed to a cleaner  
flotation, said minor fraction of feed being suffi-  
25 cient to insure the utilization of the excess pro-  
moter and the settling of substantially all the  
mineral in the rougher flotation overflow, and  
returning the cleaner flotation underflow to the  
roughest flotation feed.

HARRY L. MEAD.  
ERNEST J. MAUST.